

## UNITED STATES PATENT OFFICE

MICHAEL G. MINAEFF, OF BROOKLYN, NEW YORK, ASSIGNOR TO THE LARVEX CORPORATION, OF NEW YORK, N. Y., A CORPORATION OF NEW YORK

## MOTHPROOFING MATERIAL

No Drawing.

Application filed November 29, 1927. Serial No. 236,584.

This invention relates to the mothproofing of materials or fabrics containing animal fibres, including those known as wool, by treating them with thiourea, or certain of its derivatives, in which at least one of the amino groups contains no radical substituted for hydrogen.

It has been found that when the ordinary woolen fabric of commerce is immersed in a suitable solution of thiourea or phenylthiourea dissolved in acetone, water or other suitable solvents, it becomes immune from attack by moth larvae, such as normally attack and destroy woolen materials under similar conditions.

A two percent solution has been found entirely satisfactory, although a concentration of one percent, or even less, of thiourea, gives marked protection from moth attack. It was found that long immersion was unnecessary, and that the fabric was not affected in any degree, except for its immunity to its attack by moth larvae. In other words neither the feel nor the appearance of the fibres was sensibly altered.

In some cases it is advisable to include another substance or substances, especially such as will facilitate the wetting of the woolen material to be mothproofed. This may be advantageous whether the material is mothproofed by spraying or by immersion.

*Example.*—A solution was prepared by dissolving two parts of thiourea in a mixture of 88 parts of water and 12 parts of acetone. To this solution was added .3 parts of sulphonated castor oil, making a practically non-inflammable liquid of an entirely satisfactory wetting power. The fabric was immersed in the final solution, the excess liquid squeezed out, and the material air dried. It was then placed in a container with living moth larvae under conditions that normally result in complete destruction of the fabric by the larvae. It was found that under these conditions the fabric was practically undam-

aged by the larvae. The same fabric, except that it received no treatment with thiourea, was subjected to the action of moth larvae under identical conditions, with the result that it was completely destroyed.

Identical fabric was also destroyed when it was subjected to similar larvae test after treatment with the substituted thiourea containing a phenyl group in each amino group (thiocarbanlide).

Having thus described certain embodiments of my invention, what I claim is:

1. The process of moth-proofing material which consists in treating it with a thiourea in solution in which at least one of the amino groups contains no radical substituted for hydrogen.

2. The process of moth-proofing animal fibres which consists in treating it with thiourea in solution in such proportion that the fibres are substantially unaltered in appearance.

3. The process of moth-proofing material which consists in treating it with a solution carrying a thiourea in which at least one of the amino groups contains no radical substituted for hydrogen, the solution also containing a substance which facilitates wetting of the material by the solution.

4. The process of moth-proofing material which consists in treating it with an aqueous solution carrying a thiourea in which at least one of the amino groups contains no radical substituted for hydrogen, the solution also carrying sulphonated material.

5. A moth-proofing solution consisting of water carrying a thiourea in which at least one of the amino groups contains no radical substituted for hydrogen, and also carrying a substance which facilitates the wetting of the material by the solution.

6. A moth-proofing solution consisting of water carrying thiourea, and also carrying a substance which facilitates the wetting of the material by the solution.

50

55

60

65

70

75

80

85

90

7. An article largely consisting of animal fibres impregnated with a thiourea in which at least one of the amino groups contains no substitute for hydrogen and in such an amount that neither the feel nor the appearance of the fibres indicates that they have been so impregnated.

Signed at 250 Park Ave., in the county of New York and State of New York this 25th  
**10** day of November, A. D. 1927.

**MICHAEL G. MINAEFF.**

**15****20****25****30****35****40****45****50****55****60****65**